

April 24, 1962

J. H. BEYER ET AL

3,031,371

PAPER OF IMPROVED STRENGTH

Filed June 16, 1959



INVENTORS

J. H. Beyer  
J. H. Foreman  
L. R. Parsons

By

Watson, Cope,  
Quinle & Watson  
ATTORNEYS

# United States Patent Office

3,031,371

Patented Apr. 24, 1962

1

3,031,371

## PAPER OF IMPROVED STRENGTH

John H. Beyer, Memphis, Tenn., John H. Foreman, Cincinnati, Ohio, and Lawrence R. Parks, Memphis, Tenn., assignors to The Buckeye Cellulose Corporation, Cincinnati, Ohio, a corporation of Ohio

Filed June 16, 1959, Ser. No. 820,751

2 Claims. (Cl. 162—146)

This invention relates to improvements in the manufacture of fine papers from furnishes containing cotton fibers and more particularly is concerned with the provision of novel compositions containing the shorter fibers of the cotton plant, namely first-cut and second-cut linters, which contribute superior strength and conversion characteristics to papers formed from furnishes comprised entirely of the aforementioned compositions. In addition, the invention provides for the preparation of hydroxyethyl cellulose according to certain definite process conditions which markedly and unexpectedly improve the ability of cotton linters blends of modified and unmodified fibers to be processed into fine papers such as the bond and ledger types which heretofore have required a predominant proportion of rag stock in their furnishes in order to develop the requisite strength characteristics.

In recent years the steadily increasing use of synthetic fibers in textiles and in fabrics which in prior years had been composed entirely of staple cotton fibers has posed a serious economic and supply problem to the manufacturers of fine papers. Not only has the available supply of cotton rag stock such as shirt clippings been high in price and insufficient to meet the paper manufacturer's quantity requirements, but there has been the ever present likelihood of carrying thermoplastic and other synthetic fibers and deleterious substances into the papermaking process together with the rag stock to cause translucent spots and other quality defects intolerable in fine papers. Due to the serious nature of the problem and the apparent long term trend toward the ever increasing use of fabrics either consisting of a blend of synthetic with natural fibers or of natural fibers subjected to a variety of surface treatments, the paper manufacturers have carried on an intensive effort to develop sources of fibers suitable for their needs without deleterious admixture of unwanted fibers and substances.

It is natural that the paper industry should have considered the linters bleaching industry as a possible source of cotton fiber for their use since this source represented a large supply of pure cotton fibers in a related industry, but certain formidable problems which are the concern of this invention had to be met before this was possible. Stated in their bare essence these difficulties all revolved around the problem of processing short linters fibers, averaging 2 to 5 mm. in length, so that they would develop the strength characteristics of the longer rag stock fibers, which exceed one-half inch in length.

In general, applicants' solution to this problem, as indicated above, embodies the use of hydroxyethyl cellulose prepared from cotton linters under especially controlled conditions to produce a product having unique binding properties for the unmodified cotton linters with which it is combined in providing the furnish.

In order to appreciate the full significance of the contribution to the art of papermaking by the invention disclosed herein and to properly differentiate it from the prior art, it is necessary to review the use made heretofore in the papermaking industry of hydroxyethyl modified fibers and to understand the change in fiber properties effected by increasing levels of hydroxyethyl modification.

It is well known to prepare alkali cellulose by steeping cellulose with a sodium hydroxide solution and to react

2

the resulting alkali cellulose with ethylene oxide to produce hydroxyethyl cellulose (HEC) according to the following general formula where  $R_{cell}OH$  represents cellulose:



Likewise the treatment of cellulose with ethylene chlorohydrin to produce hydroxyethylcellulose is a well-known chemical reaction.

10 The resulting hydroxyethyl cellulose, depending on the method and conditions of preparation, may be roughly classified by its solubility in water and solutions containing 6 to 10 percent of sodium hydroxide into one of three groups, (1) water insoluble alkali insoluble, (2) water insoluble alkali soluble and (3) water soluble, the listing being given in order of increased modification of the cellulose molecule. It is known that the group to which a particular sample of hydroxyethyl cellulose will belong is dependent to a major degree on the degree of 15 substitution of its available hydroxyl groups with the hydroxyethyl group and to a minor degree on the physical treatment accorded the alkali cellulose during the modification reaction.

20 Thus HEC having a degree of substitution from .01—.25 is generally insoluble in both water and weak alkali solutions, HEC having a degree of substitution from 0.2 to 0.4 is alkali soluble and water insoluble and HEC having a degree of substitution from 0.4 to the upper limit of three hydroxyl groups available for substitution 30 is water soluble. As the degree of substitution increases toward the upper limit the individual cellulose fibers of the product HEC become increasingly swollen, and finally lose their fibrous character entirely in the water soluble range of substitution.

35 It is generally known to incorporate hydroxyethyl cellulose from all three of the substituent groups into paper furnishes for the purpose of decreasing beating time to reach a given freeness, or relative drainage speed on a wire screen, in paper stock preparation. HEC has also 40 been utilized for the purpose of generally increasing strength characteristics of the finished paper such as evidenced by the testing procedures generally in use in the paper industry for the measurement of the bursting, tensile and fold values of paper. HEC has also been 45 incorporated in paper as a sizing material. However, the present invention is not concerned with these examples of prior art but with the discovery that the steeping condition whereby the intermediate alkali cellulose is prepared is a controlling factor in the ultimate strength 50 of papers formed from blends containing the HEC prepared therefrom.

55 Heretofore the improvement in paper stock preparation or final paper strength characteristics engendered by the incorporation of HEC into a paper stock had been thought to be roughly dependent on the amount of HEC addition, a marked rapid improvement resulting when the amount added is small and extending upward to a limit past which further HEC addition produced no gain in paper strength properties.

60 It has presently been discovered, however, that these assumptions based on the prior art are incorrect and that, as more fully set forth hereinafter, a certain HEC prepared from short fibered cotton linters within critical relationships of process conditions, particularly as regards the caustic strength and temperature relationship involved in the processing of the intermediate alkali cellulose will, when incorporated with unmodified cotton linters, enable the attainment of strength characteristics in papers formed therefrom which are markedly superior to other HEC incorporated.

70 It is therefore an object of this invention to provide cotton linter fibers which are modified by substitution

under critical process conditions so that they contribute strength characteristics to paper which are markedly superior to strength improvements engendered by incorporating HEC prepared at other processing conditions.

It is a further object of the invention to provide a novel composition of hydroxyethyl modified bleached cotton linters with unmodified bleached cotton linters which will serve as a papermaking stock for the production of all cotton linter fiber papers. These papers have strength characteristics enabling them to replace rag stock papers and the strength characteristics of these papers are markedly superior to papers formed from blends in which the HEC fiber portion was processed under other conditions.

It is a still further object of this invention to provide a blend of hydroxyethyl modified bleached cotton linters with unmodified bleached cotton linters which blend is suitable for substitution as a major portion of the rag stock requirement in the furnish of fine rag stock papers.

Further objects and features of the invention will be apparent from the following description of the preferred practice thereof, and from the accompanying drawing in which FIGURES 1, 2 and 3 present graphical illustrations of the data tabulated in the examples, illustrating the unexpected and markedly superior strength characteristics induced in all cotton linter fiber papers by addition of the particular hydroxyethylated short cotton fibers described herein.

The results plotted in the drawing as further explained hereinafter in Example I were obtained by beating blends composed of 20 percent second-cut linters HEC prepared from alkali cellulose steeped at varying caustic concentrations and 80 percent unmodified first-cut linters to a Canadian Standard freeness of 200 cubic centimeters as determined by TAPPI standard method T227m-58, in an ordinary Noble & Wood 5 pound cycle beater with brass tackle. This beater is widely used in the paper industry to standardize physical tests in the laboratory since the Mullen and MIT fold of paper will vary with the freeness developed by beating the fibers of which it is composed. The blend was then made into sheets of paper for testing by TAPPI standard method T205m-58 with the exception that 75 gram per square meter sheets were produced instead of 60 gram sheets. The prepared and conditioned sheets were then tested according to TAPPI standard methods to obtain the values for Mullen and MIT fold.

In the production of bleached cotton linters, the linters are first separated from extraneous dirt, metallic matter, and field debris by hydraulic and/or mechanical means. Next, to aid in the removal of oils and waxes, the linters are digested (cooked) in digesters of various types, such as the vertical stationary or spherical rotary types, using as a digestive liquor a dilute aqueous solution of sodium hydroxide generally having a concentration of three percent, or less, to which may be added small amounts of various soaping or wetting agents, the total amount of solution used being sufficient to supply an amount of sodium hydroxide equivalent to 5-10 percent of the weight of fibers in a digester. Digestion is accomplished by subjecting the linters together with the digestive liquor to a temperature and pressure of 50 to 125 p.s.i.g. steam over a period ranging from 3 to 8 hours. Subsequent to digestion and washing, the partially purified linters are bleached with chlorine. The bleaching agent may be added to the linters in the form of chlorine gas or sodium hypochlorite in one or more stages to bleach the product to the white color of the finished product. After washing and drying, the material is the bleached cotton linters referred to herein.

The modified cotton linter fibers of this invention are prepared by taking as a starting material a quantity of cotton linters digested and bleached in the aforementioned manner, which is not a part of this invention, to a cupra-ammonium viscosity of 400-600 seconds as determined by the A.C.S. cupra-ammonium hydroxide method using a 2.5 gram sample. It is emphasized that linters pulp of

the viscosity range mentioned, although suitable in every way for the practice of the present invention, is not a part of the invention and linter pulps of any viscosity otherwise usable as paper fibers may be utilized. The alkali cellulose is then prepared by first steeping the linters in caustic alkali solution at selected temperatures, the caustic concentration and temperature being chosen to result in complete conversion to alkali cellulose with minimum degradation of the cellulose. For example, at room temperatures of the order of 20-30° centigrade, the desired conversion is achieved by steeping for 15-35 minutes in caustic of 13.5-14.5 percent strength. Although the specific examples given as illustrative of this invention refer to conventional sheet steeping, it is not intended to limit the scope of this invention thereby and the alkali cellulose may be prepared by the well-known slurry process for converting bulk cellulose to alkali cellulose provided the processing conditions specified above are maintained as to time, temperature and caustic strength.

The steeped pulp is then drained of caustic solution and pressed so that the weight ratio of the cotton linter fibers plus the retained steeping caustic to that of the bone dry weight of the original fibers is about 3.

The resulting alkali cellulose cake is then reduced to 20 crumb form in a suitable shredder such as a sigma blade mixer. After shredding, or crumbling, the alkali cellulose crumbs are placed in a closed reactor which is then evacuated, blanketed with nitrogen and reevacuated to 25 eliminate the danger of explosion. Gaseous ethylene oxide is then introduced into the reactor until about 20% to 30% by weight based on the bone dry weight of the original bleached second-cut cotton linter fibers has been added. The rate of addition is adjusted so that a maximum pressure of 25 inches of mercury is maintained 35 within the reactor during the period of ethylene oxide addition and so that the temperature of the pulp mass does not exceed 70 degrees centigrade. The modified linter fibers are allowed to remain within the sealed reactor for 20 to 30 minutes following the period of ethylene oxide addition.

The modified linter fiber product of the reaction is then 40 discharged from the reactor and repulped with water to a consistency of between 2% and 5% and sufficient mineral acid, such as 10% sulphuric acid, is added to neutralize the sodium hydroxide carried with the modified fibers and so that the pH of the fiber slurry is adjusted to between 45 5 and 8.

As hereinbefore stated it is known to incorporate hydroxyethyl cellulose of various degrees of substitution and prepared by any of the reactions of the prior art into paper furnishes. The present invention is therefore not concerned with the general scheme of HEC production but with the discovery and reduction to practice of a relationship in the production of alkali cellulose for subsequent use in HEC paper furnishes which greatly enhances the strength of papers produced from blends of modified and unmodified cotton linters. Accordingly it is found that alkali cellulose prepared by treating cotton linters fibers with 13.5 to 14.5 percent aqueous sodium hydroxide solution at 25° centigrade and thereafter pressing the treated cellulose to a press weight ratio of about 60 3 will result in the unexpected strength increases in paper strength attributable to the practice of this invention when the resulting alkali cellulose is converted to HEC and used in a blend with unmodified cotton linter fibers in a 65 paper furnish. Although the 25° centigrade 13.5 to 14.5 percent caustic steep is the presently preferred mode of operation, it is not intended to thus limit the invention and other operable caustic strength-temperature relationships are known to exist.

Sufficient unmodified bleached cotton linters to result 70 in a blend of 10 to 30 percent modified fibers and 70 to 90 percent unmodified fibers is added to the slurry while water is added to maintain the pumpable consistency of the slurry.

Subsequent to this operation the slurry may be pumped directly to stock preparation equipment such as beaters or jordans and then to the paper machine for sheeting. Alternatively it may be dewatered and dried for handling reasons and supplied to a paper manufacturer in either bulk or sheet form as a suitable stock for an all cotton fiber paper.

The preferred mode of practicing the invention is described more particularly in the following examples, but it will be understood that limitation of the scope of the invention is not thereby intended.

#### EXAMPLE I

A 135 pound portion of 500 second cuprammonium viscosity (based on the standard A.C.S. determination for viscosity using a 2.5 gram sample) second-cut cotton linter pulp sheets were placed in a vertical position in a viscose steeping press. These sheets were 19.5" x 21" x .045" with the sheets cut with their long dimensions parallel to the grain or in the machine direction. An aqueous 14% caustic solution was introduced at the bottom of the press at a rate which minimized floating and wicking, i.e. at a rate so that the rise in caustic level was approximately equal to the rise of the caustic solution in the sheets induced by capillarity. The temperature of the caustic steeping solution was maintained at 25 degrees centigrade and the pulp sheets remained submerged for 20 minutes.

Following this period of steeping in 14% caustic, the caustic solution was drained from the pulp sheets and the ram of the steeping press was advanced to press the sheets to a cellulose content of 33 1/3%, i.e. to a press weight ratio of 3.

The resulting alkali cellulose was shredded in a sigma blade type shredder and immediately charged into a reactor capable of being sealed from the atmosphere, which in this instance was a viscose type barette.

To safeguard against the explosive hazards of ethylene oxide reactions, the reactor was evacuated to a pressure of 25 inches of mercury whereupon nitrogen was introduced to bring the reactor up to atmospheric pressure. After this flushing precaution the reactor was sealed and again evacuated.

Gaseous ethylene oxide was added to the charged alkali cotton linters cellulose at a rate whereby the reaction maintained a pressure of 25 inches of mercury within the barette reactor and the temperature of the pulp mass did not exceed 70 degrees centigrade until the amount of ethylene oxide charged was equal to 25% of the weight of the original bone dry weight of the cotton linters placed in the steeping press. The reacted linters were allowed to remain in the reactor for a period of 20 minutes following the addition of the prescribed amount of ethylene oxide.

The hydroxyethyl modified second-cut cotton linters were then removed from the reactor and blended with unmodified bleached first-cut cotton linters in water to give a 20% blend of the modified linters together with 80% of the unmodified linters, the percentage being calculated on a cellulose basis neglecting any increase in weight of the modified fibers due to the reaction with ethylene oxide.

The consistency of the slurry was adjusted to 3% of pulp in water and 10% sulphuric acid was added to neutralize the sodium hydroxide introduced with the reacted fiber and adjust the pH of the slurry to 7.

The resulting blend was then jordaned to a Canadian Standard freeness of 750 to 800 cubic centimeters in order to decrease the beating time of the blend and to facilitate sheet formation. The Williams freeness test is widely used in the pulp and paper industry as an empirical measurement of the rate at which a dilute suspension of pulp may be partially dewatered and is indicative of the fibrillation and/or the degree and manner of the subdivision of the individual fibers in pulp. For testing purposes handsheets were made according to TAPPI Standard

method number T205m-58 with the exception of the sheet weight which was 75 grams per square meter. Mullen was determined according to TAPPI Standard method T403m-58, tear strength according to T414m-49, tensile strength according to T404m-50, and MIT fold according to T423m-50-II.

In a similar fashion other experimental runs were made varying the percentage strength of the steeping caustic while holding the other variables within the limits of experimental error. The conditions and results of these experimental runs are tabulated in the following Table I. The information is also presented graphically in the attached drawing to show the superiority of blends in which the hydroxyethyl cellulose modified portion was produced under the conditions of this invention.

Table I

#### RESULTS AT 200 CC. CANADIAN STANDARD

| Percent<br>NaOH<br>in Steep | Steep<br>Temp.,<br>° C. | Press<br>Weight<br>Ratio | Beating<br>Time,<br>Minutes | Mullen,<br>lbs./<br>sq. in. | Tear<br>Grams<br>Per<br>Sheet | MIT<br>Fold<br>Num-<br>ber<br>Double<br>Folds | Tens.<br>lbs./<br>inch<br>Test<br>Strip<br>Width |
|-----------------------------|-------------------------|--------------------------|-----------------------------|-----------------------------|-------------------------------|-----------------------------------------------|--------------------------------------------------|
| 25                          |                         |                          |                             |                             |                               |                                               |                                                  |
| 7.79                        | 24                      | 2.80                     | 61                          | 39                          | 102                           | 225                                           | 22                                               |
| 2.79                        | 37                      | 2.60                     | 57                          | 37                          | 101                           | 180                                           | 26                                               |
| 11.30                       | 34                      | 2.74                     | 48                          | 45                          | 103                           | 380                                           | 23                                               |
| 11.30                       | 26                      | 2.62                     | 50                          | 43                          | 102                           | 290                                           | 24                                               |
| 13.08                       | 25                      | 3.05                     | 39                          | 54                          | 93                            | 850                                           | 27                                               |
| 13.08                       | 37                      | 2.80                     | 40                          | 50                          | 99                            | 740                                           | 26                                               |
| 14.00                       | 25                      | 3.0                      | 39                          | 56                          | 103                           | 942                                           | 26                                               |
| 14.50                       | 34                      | 2.80                     | 27                          | 54                          | 102                           | 820                                           | 25                                               |
| 14.50                       | 26                      | 3.02                     | 29                          | 53                          | 103                           | 660                                           | 28                                               |
| 16.98                       | 26                      | 3.07                     | 32                          | 45                          | 100                           | 390                                           | 24                                               |
| 17.00                       | 26                      | 3.04                     | 30                          | 47                          | 99                            | 550                                           | 26                                               |
| 17.06                       | 34                      | 3.05                     | 29                          | 47                          | 97                            | 530                                           | 25                                               |
| 35                          |                         |                          |                             |                             |                               |                                               |                                                  |
| 17.64                       | 34                      | 2.97                     | 27                          | 46                          | 100                           | 530                                           | 23                                               |
| 22.71                       | 27                      | 3.03                     | 30                          | 45                          | 102                           | 375                                           | 23                                               |
| 22.71                       | 34                      | 3.02                     | 31                          | 43                          | 108                           | 380                                           | 27                                               |
| 26.94                       | 25                      | 3.01                     | 33                          | 46                          | 101                           | 310                                           | 23                                               |
| 26.94                       | 40                      | 3.06                     | 30                          | 47                          | 100                           | 410                                           | 23                                               |
| 30.52                       | 36                      | 3.02                     | 32                          | 40                          | 104                           | 330                                           | 23                                               |
| 30.52                       | 27                      | 3.07                     | 31                          | 42                          | 102                           | 240                                           | 22                                               |

The graphs of the above data appearing in the drawing as FIGURES 1, 2 and 3 illustrate the minimum beating time, and sharp increase of paper strength characteristics resulting from the use in blends of the modified linters fibers of this invention in comparison with blends utilizing modified linter fibers prepared by other processing conditions. FIGURE 1 compares the beating times for blends to reach a Canadian Standard freeness of 200 cubic centimeters with the caustic strength at which the linters of the modified portion of the blend was steeped in order to convert them to alkali cellulose. In a similar fashion FIGURES 2 and 3 compare MIT fold and Mullen values respectively with the concentration of steeping caustic used in preparing the modified portions of the blend.

Although the present invention is best described by the results obtained from the use of the herein defined modified fiber product and blend as the sole furnish in the cotton linter paper, it is not intended to limit the scope of the invention thereby and it is pointed out that addition of the HEC and blends of this invention will improve the strength characteristics of papers produced from even the best rag stock furnishes. Also, it is considered that all of the possible combinations of modified first and second-cut linters prepared according to the methods described herein together with unmodified first and second-cut linters be within the scope of the invention. Furthermore, it has been ascertained that 14 percent sodium hydroxide is the minimum strength aqueous sodium hydroxide solution which will effect the conversion of cotton linter cellulose to cellulose-II (alkali cellulose) at the specified temperature of about 25 degrees centigrade.

The following table gives examples of the temperature-percentage relationships where the strength of the

sodium hydroxide is the minimum to effect the conversion of cotton linter cellulose to cellulose-II.

| Temperature, degrees centigrade: | Percentage, sodium hydroxide |
|----------------------------------|------------------------------|
| 5                                | 11                           |
| 15                               | 13                           |
| 25                               | 14                           |
| 35                               | 16                           |
| 45                               | 17                           |

It is emphasized that the above enumerated relationships do not relate all of the temperature percentage steeping combinations resulting in the improved capacity of the HEC produced from alkali cellulose steeped at the conditions to impart improved strength characteristics to paper. In fact an infinite number of such relationships exist at temperatures above, between, and below those cited and HEC produced at any of the relationships as hereinbefore defined will be found to have superior properties as a paper additive.

Having thus described the invention, what is claimed as new and desired to be secured by Letters Patent is:

1. A modified bleached cotton linter product produced by steeping purified and bleached short fibered cotton linters in the minimum concentration of aqueous sodium hydroxide which will convert the fibers to alkali cellulose at a given temperature for about 15 to 35 minutes, draining the aqueous sodium hydroxide solution from the fibers, pressing said fibers so that the ratio of the weight of fibers together with the retained sodium hydroxide solution to the bone dry weight of the original

fibers is about 3 and reacting the so-treated fibers with about 20% to about 30% by weight of ethylene oxide based on the bone dry weight of the original fibers, said modified cotton linter product contributing superior beating, bursting and folding characteristics to paper furnishes and papers composed of all cotton fibers when added thereto in amounts of about 10% to about 30% by weight of the fiber stock contained in the furnish.

2. As a new composition of matter, a blend of bleached cotton linter fibers suitable for a paper furnish comprised of about 10% to about 30% by weight of bleached cotton linter fibers modified by treatment with ethylene oxide comingled with about 90% to about 70% of unmodified bleached cotton linter fibers, the hydroxyethylation of the modified portion of said blend including the step of steeping bleached cotton linter fibers in the minimum concentration of aqueous sodium hydroxide which will convert the fibers to alkali cellulose at a given temperature for about 15 to about 35 minutes.

20

References Cited in the file of this patent

UNITED STATES PATENTS

|           |                  |               |
|-----------|------------------|---------------|
| 1,857,100 | McCormick et al. | May 3, 1932   |
| 2,488,631 | Kunz             | Nov. 22, 1949 |
| 2,533,145 | Schorger         | Dec. 5, 1950  |
| 2,572,039 | Klug et al.      | Oct. 23, 1951 |
| 2,682,535 | Broderick        | June 29, 1954 |
| 2,736,653 | Erickson         | Feb. 28, 1956 |
| 2,833,614 | Kersnar          | May 6, 1958   |
| 2,847,411 | Mitchell et al.  | Aug. 12, 1958 |
| 2,916,413 | Harpham          | Dec. 8, 1959  |

25

30